

Oct. 22, 1935.

G. P. HALLIWELL

2,018,520

HIGH STRENGTH ALLOY

Filed March 3, 1932

2 Sheets-Sheet 1

Fig. 1



Fig. 2.



WITNESSES:

Arthur J. McManon  
Mrs. C. Groome

INVENTOR

George P. Halliwell.  
BY Howard Flint.

ATTORNEY

Oct. 22, 1935.

G. P. HALLIWELL

2,018,520

HIGH STRENGTH ALLOY

Filed March 3, 1932

2 Sheets-Sheet 2

Fig. 3.



Fig. 4.



Fig. 5.



WITNESSES:

Patrick J. McMahon  
John C. Groome

INVENTOR

George P. Halliwell.

BY Howard Flint.

ATTORNEY

## UNITED STATES PATENT OFFICE

2,018,520

## HIGH STRENGTH ALLOY

George P. Halliwell, Wilkinsburg, Pa., assignor to  
Westinghouse Electric & Manufacturing Company, a corporation of Pennsylvania

Application March 3, 1932, Serial No. 596,565

4 Claims. (Cl. 148—13)

My invention relates to alloys and more particularly to alloys having a comparatively high strength at elevated temperatures.

The principal object of my invention is to provide an alloy containing nickel, cobalt, iron and titanium which is characterized by having a high proportional limit and a high tensile strength at normal and elevated temperatures.

Another object of my invention is to provide an alloy containing nickel, cobalt, iron and titanium which has been subjected to a specific ageing process whereby the characteristics of the alloy are substantially changed and an alloy having greatly improved physical properties is produced.

A still further object of my invention is to provide alloys and a process of producing alloys containing cobalt, iron and titanium; nickel, cobalt and titanium; nickel, iron and titanium; or nickel, cobalt, iron and titanium, which comprises quenching the alloy from a comparatively high temperature and then subjecting it to an ageing process at a lower temperature for a sufficient length of time to improve its physical properties.

It has heretofore been customary to utilize a metal, such as iron or steel, for the component parts of power plant apparatus, such as super-heaters, steam boilers, turbines, and turbine blades. Since the limiting temperatures and pressures at which such apparatus can be operated, however, are governed largely by the tensile strength and proportional limit of the material of which they are composed, it is essential that the metal or alloy utilized shall have a high tensile strength and retain its initial dimensions under stress.

I have made the discovery that if alloys containing cobalt, nickel, iron and titanium are quenched from a comparatively high temperature, such as 900° C. to 1000° C., and then subjected to an ageing process at a lower temperature for varying lengths of time, the proportional limit and tensile strength of the alloy at normal and elevated temperatures will be substantially improved.

My improved alloy has a proportional limit and an ultimate tensile strength that is far superior to that of steel or of ferrous or non-ferrous alloys which have heretofore been utilized for such purposes. The fact that these physical properties are maintained at elevated temperatures also renders it especially suitable for use as the contacting portions of valves and valve seats for internal combustion engines or for valves of

other machines or apparatus which are operated at comparatively high temperatures. Its high tensile strength and resistance to oxidation at comparatively high temperatures also renders it especially valuable for use in springs and other apparatus. 5

My improved alloy comprises nickel, cobalt, iron and titanium in various proportions and may also contain chromium, although satisfactory results have been obtained when the chromium is omitted. The respective proportions of iron, nickel and cobalt which are present in the alloy may be varied over wide ranges and, if desired, either the cobalt, nickel or iron may be entirely omitted, although the physical characteristics of the alloy will not be as satisfactory as when all the elements are present. 10

In order that the alloy may be forgeable, it is also essential that the titanium should be maintained below 10% and preferably below 7%. As 20 a rule I prefer to utilize amounts ranging from 2% to 5%. I also find it very desirable to have nickel present in substantial amounts to minimize oxidation. I also find that nickel greatly improves the physical properties of the alloy at 25 normal and elevated temperatures.

In general, it may be stated that the nickel may range from more than incidental impurities up to 70%, the cobalt from 10% to 80%, the iron from 5% to 60%, and the titanium from .5% 30 to 10%, and chromium may be present in amounts ranging from more than incidental impurities up to 25%. Carbon may also be present in limited amounts but is preferably maintained 35 below 1%.

Better results may be obtained when the nickel is maintained in amounts ranging from 20% to 70%, cobalt in amounts ranging from 10% to 60%, iron in amounts ranging from 5% to 50%, and titanium ranging in amounts from 40 2% to 5%.

In the preferred embodiment of my invention, the base of nickel plus cobalt constitutes the major proportion of the alloy, and the amount of nickel is greater than the amount of cobalt. 45 For example, the nickel is preferably maintained in amount from 40% to 60%, cobalt in amount ranging from 20% to 35%, iron in amount ranging from 5% to 20%, and the titanium in amount ranging from 2% to 5%. I have also found it 50 very desirable to have chromium present in amounts ranging from 1% to 25%.

In preparing my improved alloy, the nickel and cobalt are first melted together in a reducing or inert atmosphere and the additional al- 55

loying ingredients are then added. I prefer to add the iron and titanium in the form of a ferro-titanium alloy containing approximately 75% iron and 25% titanium, though to obtain desired percentage of iron or titanium, additional amounts of either one of these metals may be added in the elementary form. After the melt is completed and just before casting, a small amount, say from one to two grams, of a de-oxidizer, such as aluminum, silicon or manganese, is attached to a rod composed of nickel or of a cobalt-nickel base alloy, and plunged into the molten bath. Care should be exercised in introducing the deoxidizer as it causes a rapid reaction of almost explosive violence.

The alloys are next cast, homogenized (at 1000° C. for 8 hours), forged and annealed at a temperature of from 900° C. to 1000° C. for approximately one hour and quenched from that temperature. The quenching may be accomplished by any suitable cooling medium, such as air, oil or water. The alloys are then subjected to an ageing process at temperatures of from 500° C. to 800° C. for a period of time ranging from  $\frac{1}{2}$  to 2,000 hours. In general, it may be stated that the greatest improvement in the characteristics of the alloy which is effected by the ageing process takes place within the first few hours, and that about 80% of the maximum increase in hardness is effected after 72 hours. The time of ageing is also dependent upon the ageing temperature. At higher temperatures the ageing takes place in a shorter period of time. After the alloy has aged for a sufficient time to produce the maximum hardness, the alloy is cooled.

The increase in hardness that may be imparted to my improved alloys and their ability to retain their initial dimensions under stress at high temperatures will be better understood by reference to the accompanying drawings, in which

Figure 1 is a graph showing the increased hardness that may be imparted to my improved alloys by ageing at a temperature of 600° C.;

Figs. 2 and 3 are similar graphs showing the effects of ageing at temperatures of 650° C. and 750° C., respectively;

Fig. 4 is a graph showing the resistance to strain of my improved alloys as compared to carbon steel containing approximately .5% carbon; and

Fig. 5 is a graph similar to Fig. 4 showing the resistance to strain of my improved alloys as compared to a nichrome alloy containing approximately 60% nickel, 20% iron, 18% chromium, and 2% manganese.

In Figs. 1, 2 and 3 of the drawings, the ordinates represent hardness as measured in Vickers Pyramid Numerals and the abscissae represent time of ageing in hours. In these figures the numerals 1 to 12, inclusive, are representative alloys having approximately the following compositions:

|    | Nickel | Cobalt | Iron | Titanium | Chromium | Carbon |
|----|--------|--------|------|----------|----------|--------|
| 1  | 19.5   | 78     |      | 2.3      |          |        |
| 2  | 23     | 40     | 34   | 2.23     |          | .08    |
| 3  | 49     | 29.5   | 8.4  | 2.4      | 9.5      | .02    |
| 4  | 5      | 19     | 72   | 2.5      |          |        |
| 5  | 57     | 27     | 10   | 4.3      |          |        |
| 6  | 20     | 20     | 57.5 | 2.5      |          | .07    |
| 7  |        | 60     | 37.5 | 2.5      |          |        |
| 8  | 73.3   | 17.3   | 6.25 | 2.4      |          |        |
| 9  | 46.9   | 29.5   | 6.5  | 2.35     | 13.7     |        |
| 10 | 13     | 41     | 43.5 | 2.5      |          |        |
| 11 | 46.1   | 24.9   | 7.0  | 2.2      | 18.74    |        |
| 12 | 22     | 19     | 56.5 | 2.5      |          |        |

The increase in hardness of the alloy is undoubtedly caused at least partially by the precipitation of titanium either alone or as a compound of one or more of the alloying ingredients from solid solution during the ageing process. My experiments indicate, however, that unless substantial quantities of iron and cobalt are present, a pronounced increase in hardness will not be obtained at ageing temperatures.

From Figs. 1, 2 and 3 of the drawings, it will also be apparent that when the nickel and cobalt constitute the major proportion of the alloy, the ageing will be very rapid and the hardness attained will be comparatively high. This is indicated from alloys designated by the curves 5, 7, 9 and 10. I, therefore, prefer that the nickel plus cobalt content shall constitute at least a major proportion of the alloy. It will be noted, however, that the alloy represented by curve 7 does not contain any nickel which indicates that my process is also applicable to alloys containing cobalt, iron and titanium. The physical properties of such alloys, however, are not as good as when nickel is present.

In Figs. 4 and 5 of the drawings, in which the ordinates designate percentage of maximum deflection and the abscissae represent the temperature, curves illustrative of representative alloys indicate the superiority of my improved alloys over medium carbon steel and nichrome in retaining their initial dimensions under stress. This property is highly important in alloys employed for service at high temperatures.

In making tests to determine this characteristic, the alloys were first rolled down to a thickness of about .017 of an inch, cut into strips  $5\frac{1}{2}$  inches in length, heated at a temperature of 950° C. for a period of 30 minutes, and cooled rapidly. The alloys were next subjected to my improved ageing process at a temperature of 650° C. for a 40 period of 72 hours.

The flat strips were then placed in a form of known radius and maintained 30 minutes at the desired temperature. After cooling, the strips were removed from the form and laid across two pivots placed four inches apart. The bend produced was measured by determining the radius of curvature of the strip by means of a fixed micrometer at a point midway between the pivots. Since the curvature of the form is fixed, the vertical displacement in a four inch chord can be readily calculated. In the graphs shown in Figs. 4 and 5, the percentage of maximum deflection equals the vertical displacement of the strip, after being constrained for the period and at the temperature indicated and then cooled, divided by the vertical displacement of the form, and multiplied by 100.

Curves 1, 2, 3, 4, 5 and 7 in Figs. 4 and 5 designate alloys having the same composition as the corresponding curves in Figs. 1, 2 and 3.

Curve 14 designates medium carbon steel and curve 15 a nickel-iron-chromium alloy containing approximately 60% nickel, 21% chromium, 17% iron and a small percentage of manganese, commonly referred to as nichrome.

From the drawings it will be noted that my improved alloy is far superior to carbon steel in maintaining its initial dimensions under stress and is considerably better than nichrome in this respect.

During my researches on this subject, a series of alloys were prepared in which the nickel, cobalt, iron, titanium, and in some instances chromium, were present in amounts ranging from 75

20% to 70% nickel, 0% to 60% cobalt, 5% to 60% iron, 2% to 5% titanium, and 1% to 20% chromium. The alloys after being aged at 650° C. for a period of 72 hours had a proportional limit ranging from 45,000 to 80,000 pounds per square inch at room temperature and a proportional limit ranging from 30,500 to 66,250 pounds per square inch at a temperature of 600° C. The tensile strength ranged from 135,000 to 170,250 pounds per square inch at room temperature, and 92,000 to 120,200 pounds at a temperature of 600° C. The ductility of the alloy varies considerably in accordance with the composition.

The following specific examples represent the preferred embodiment of my invention in which the proportions of nickel, cobalt, iron, titanium and chromium are within the range of 40% to 60% nickel, 20% to 35% cobalt, 5% to 20% iron, 2% to 5% titanium and 1% to 20% chromium.

| Alloy number | Composition |        |      |          |          |
|--------------|-------------|--------|------|----------|----------|
|              | Nickel      | Cobalt | Iron | Titanium | Chromium |
| 9.....       | 46.9        | 29.4   | 6.5  | 2.3      | 13.7     |
| 9a.....      | 48.9        | 29.5   | 8.4  | 2.4      | 9.5      |
| 16.....      | 48.3        | 27.3   | 20.0 | 2.7      | 0.3      |
| 11.....      | 46.1        | 24.8   | 7.0  | 2.1      | 18.7     |
| 17.....      | 57.9        | 33.1   | 6.3  | 2.6      | -----    |

The above alloys were aged at a temperature of 650° C. for a period of 72 hours and their physical properties at room temperature and at a temperature of 600° C. were determined. The following table shows their physical properties at room temperature and a temperature of 600° C.

| Alloy number | Proportional lbs. per sq. room temperature | Limit inch 600° C. | Tensile strength lbs. per sq. inch |         | Percent elongation |         |
|--------------|--------------------------------------------|--------------------|------------------------------------|---------|--------------------|---------|
|              |                                            |                    | Room temperature                   | 600° C. | Room temperature   | 600° C. |
| 9.....       | 61,250                                     | 66,250             | 160,500                            | 120,200 | 27.0               | 11.0    |
| 9a.....      | 52,500                                     | 52,500             | 170,250                            | 121,500 | 26.0               | 5.2     |
| 16.....      | 80,000                                     | 57,500             | 164,750                            | 121,000 | 29.0               | 21.5    |
| 11.....      | 70,000                                     | 57,500             | 137,100                            | 127,100 | 35.0               | 24.7    |
| 17.....      | 45,000                                     | 52,000             |                                    | 105,000 |                    |         |

From the foregoing tables it will be noted that in the preferred embodiment of my invention, the nickel plus cobalt content constitutes the major proportion of the alloy and that the amount of nickel is greater than the amount of cobalt. I do not desire, however, to be limited to an alloy in which such a ratio exists as alloys have been produced in which either the nickel or cobalt has been omitted. For example, alloy No. 7, previously referred to, does not contain any nickel and in my investigation of this subject, I have produced alloys in which the cobalt has been entirely omitted. For example, an alloy containing approximately 70% nickel, 27.5% iron and 2.5% titanium was prepared, quenched from a high temperature and aged for 72 hours at a temperature of 650° C. Upon testing the alloy at room temperature and 600° C. it was found that it had a proportional limit and tensile strength of 65,000 and 150,250 pounds per square inch at room temperature, respectively, and a proportional limit and tensile strength at 600° C. of 49,500 and 100,000 pounds per square inch, respectively.

The high proportional limit of my improved

alloys and their ability to retain their initial dimensions under stress, render them especially adaptable for use in apparatus which is subjected to high temperatures. Particular attention is directed to alloy No. 9 in the foregoing table which has a proportional limit of 66,250 pounds per square inch at a temperature of 600° C. and an elongation of 11%. Such phenomenally valuable properties have not heretofore been approached in any known alloy. The highest previous value that had been attained in cobalt-nickel base alloys which had not been subjected to an ageing process was 33,750 pounds per square inch. The marked improvement imparted to the alloys by my improved process will therefore readily be appreciated. From Figs. 4 and 5 of the drawings, it will also be apparent that my improved alloy is superior to nichrome or medium carbon steel in retaining its initial dimensions under stress.

While I have described my invention in considerable detail and have given numerous examples, it will be understood that the present invention is not limited to the specific details set forth in the foregoing examples which should be construed as illustrative and not by way of limitation, and in view of the numerous modifications which may be effected therein without departing from the spirit and scope of this invention, it is desired that only such limitations be imposed as are indicated in the appended claims.

I claim as my invention:

1. The process of improving the physical properties of an alloy containing essentially from 20% to 70% nickel, 60% to 10% cobalt, 5% to 50% iron, and 0.5% to 10% titanium, which com-

prises quenching the alloy from temperatures of at least 900° C. and ageing it at temperatures of 50° C. from 500° to 800° C. for a period of at least one-half hour.

2. The process of improving the physical properties of an alloy containing essentially from 40% to 60% nickel, 20% to 35% cobalt, 5% to 20% iron, 0.5% to 10% titanium, which comprises quenching the alloy from a temperature of at least 900° C. and ageing at temperatures ranging from 500° to 800° C. for at least one-half hour.

3. An alloy comprising essentially 20% to 70% nickel, 60% to 10% cobalt, 5% to 50% iron and 0.5% to 10% titanium, which has been quenched from a temperature of at least 900° C. and aged at a temperature of 500° to 800° C. for a period of at least one-half hour.

4. An alloy comprising essentially 40% to 60% nickel, 20% to 35% cobalt, 5% to 20% iron and 0.5% to 10% titanium, which has been quenched from a temperature of at least 900° C. and aged at a temperature of 500° to 800° C. for a period of at least one-half hour.

GEORGE P. HALLIWELL.